

## UNITED STATES PATENT OFFICE

2,182,186

## GLUE TREATMENT

Walter M. Urbain and Lloyd B. Jensen, Chicago,  
Ill., assignors to Industrial Patents Corpora-  
tion, Chicago, Ill., a corporation of Delaware

No Drawing. Application December 24, 1936,  
Serial No. 117,565

7 Claims. (Cl. 260—118)

This invention relates to the treatment of glue. It is desirable in the preparation of glue to produce a product which is light in color.

We have discovered that the combination of 5 hydrogen peroxide and a nitrate is an effective bleaching agent for use in the treatment of glue. It may be that the utility of such mixtures is dependent upon the formation of pernitric acid (HNO<sub>4</sub>).

10 We have found that the nitrites are ineffective in the bleaching of glue by reason of the property of nitrites to form a dark or reddish compound by the action of nitrites on proteins. However, nitrites do not have such an effect upon proteins, 15 and the combination of hydrogen peroxide and a nitrate is peculiarly effective in bleaching glue. We have found, for example, that although potassium nitrate has no noticeable bleaching effect on glue and hydrogen peroxide has an appreciable 20 effect, the combination of hydrogen peroxide and potassium nitrate bleaches glue to a lighter color than does hydrogen peroxide alone.

In one test of the present invention, four 25 samples of a bone glue liquor containing 31.5 per cent. solids were placed in jars, each jar containing 400 gm. of the glue liquor or 126 gm. of the glue solids. The table shows the percentage 30 of potassium nitrate and hydrogen peroxide added.

30 The hydrogen peroxide was added as 30 per cent. hydrogen peroxide. The potassium nitrate was dissolved in a small amount of water and the solution added to the liquor. The mixture was agitated to thoroughly admix the hydrogen 35 peroxide and potassium nitrate with the glue liquor. The samples were stored at about 100° F. for several hours and color comparisons made. The jelly and viscosity measurements were made three days later.

Table

| 40 | Sample | Percent potassium nitrate (solids basis) | Percent hydrogen peroxide (solids basis) | 11 per cent. basis |                          |
|----|--------|------------------------------------------|------------------------------------------|--------------------|--------------------------|
|    |        |                                          |                                          | Jelly in grams     | Viscosity in millipoises |
| 45 | 1      | 1.0                                      | 0.6                                      | 119                | 54                       |
|    | 2      | 2.0                                      | 0.6                                      | 116                | 53                       |
|    | 3      |                                          | 0.6                                      | 121                | 55                       |
| 50 | 4      |                                          |                                          | 119                | 54                       |

After the bleaching action was completed, the glue liquor was evaporated and the colors of the dry glue compared. Sample No. 2 was lightest and most desirable in color. Sample No. 1 was next in lightness. Sample No. 4 had not been bleached and Sample No. 3, although slightly bleached, was not nearly as light nor as desirable in color as Samples No. 1 and No. 2.

It will be noted that the bleaching procedure of the present invention brings about no significant changes in bloom or viscosity.

We claim:

1. The method of bleaching glue which comprises adding thereto hydrogen peroxide and a nitrate. 15
2. The method of bleaching glue which comprises adding thereto hydrogen peroxide and potassium nitrate.
3. The preparation of glue which comprises adding hydrogen peroxide and a nitrate to glue liquor, agitating the mixture to secure intimate admixture, permitting the combination of hydrogen peroxide and a nitrate to act upon the glue liquor, and thereafter drying the glue liquor. 20
4. The preparation of glue which comprises adding hydrogen peroxide and potassium nitrate to glue liquor, agitating the mixture to secure intimate admixture, permitting the combination of hydrogen peroxide and potassium nitrate to act upon the glue liquor, and thereafter drying 25 the glue liquor.
5. In the manufacture of glue having a light color, the step of adding to the glue liquor a mixture of hydrogen peroxide and a nitrate. 30
6. In the manufacture of glue having a light color, the step of adding to the glue liquor a mixture of hydrogen peroxide and potassium nitrate. 35
7. In the manufacture of glue having a light color, the step of adding to the glue liquor a mixture of from 1 per cent. to 2 per cent. potassium nitrate and approximately 0.6 per cent. hydrogen peroxide, the percentages computed upon the solids basis of the glue liquor. 40

WALTER M. URBAIN.  
LLOYD B. JENSEN.